

Sept. 10, 1957

P. PAYSON

2,805,942

ALLOY STEEL AND ARTICLES THEREOF

Filed Nov. 5, 1953

*Fig. 2.*



*Fig. 3.*



*Fig. 4.*



INVENTOR.

PETER PAYSON.

BY *Ward Crosby & Keaf.*

ATTORNEYS.

1

2,805,942

**ALLOY STEEL AND ARTICLES THEREOF**

Peter Payson, New York, N. Y., assignor to Crucible Steel Company of America, Pittsburgh, Pa., a corporation of New Jersey

Application November 5, 1953, Serial No. 390,314

4 Claims. (Cl. 75—126)

This invention pertains to alloy steels which are characterized in possessing a relatively high resistance to deformation under stress at high temperatures and a good resistance to oxidation at temperatures up to about 2100° F. Moreover, this invention relates to rider sheets made of alloy steels which are suitable for use in a normalizing furnace.

In the processing of low carbon sheet steel which is made into automobile body parts, and the like, by deep drawing and forming operations, it is customary to normalize the steel before it is annealed. The normalizing is carried out in a furnace approximately 100 ft. long which may have as many as five zones each about 20 ft. long maintained at different temperatures, for example, 1725° F. at the intake end; and in succession 1800° F.; 1900° F.; 1600° F.; and finally 1325° F., at the discharge end. The hearth of the furnace consists of a series of rollers. Across the tops of the rollers are placed removable rider sheets made of heat resistant steel, and the sheets to be normalized are placed upon the rider sheets. In the normalizing operation, the sheets are moved by means of the rollers through the successive zones of the furnace at a rate of about 10 ft. per minute. The purpose of the rider sheets is to provide a support for the sheets being normalized so that they will not bend or sag between the rollers, since the sheets being normalized are sometimes very light gauge, namely, 0.022 to 0.049 in. thick, and are sufficiently weak at the high temperatures used in normalizing to sag under their own weight. The rider sheets themselves may sag somewhat in the hottest zones of the furnace, but being made of alloy heat resistant steel, and being somewhat thicker than many of the sizes of the sheets being normalized they provide sufficient support to the sheets being normalized to hold the distortion of the latter to a minimum. For ease of handling in subsequent operations it is desirable that the sheets after they have been normalized be as flat as possible.

The rider sheets are used over and over again until they become perforated or warped to such a degree that they are no longer serviceable. They are placed across the rollers at the intake end of the furnace and are removed and placed on carts at the discharge end. They are then brought back on the carts to the intake end and again placed on the rollers for another trip through the furnace. Generally the rider sheets are used only in a position below the sheets being normalized, but when sheets made from cold rolled strip are normalized, the rider sheets may be used both below and above the sheets being normalized. The purpose of the top rider sheets is to protect the sheets being normalized against excessive scaling. In successive trips through the furnace, the rider sheets are used for either top or bottom sheets interchangeably.

In the past the most satisfactory rider sheets were made from a 25% chromium-20% nickel, heat resistant steel generally designated as "Type 310, Stainless." However, because of restrictions on the use of nickel in steels

2

for non-military applications, Type 310 steel is no longer available for rider sheets and the plain 25% chromium steel generally designated "Type 446 Stainless" has been used as a substitute. Because Type 446 has a structure consisting primarily of ferrite and carbides, in contrast to the structure of austenite and carbides in Type 310, the sheets made from Type 446 are much weaker than those made from Type 310. As is well known, austenite is much stronger than ferrite at temperatures above about 1200° F. The rider sheets made from Type 446 stretch appreciably in service because of this weakness, and have to be sheared from time to time to get them back to their original dimensions in length and width. They also perforate more rapidly than the Type 310 sheets because of this attenuation. Consequently, the lives of the Type 446 sheets are only 35 to 50% as long as those of the Type 310 sheets, and the operators of these normalizing furnaces have demanded a steel for rider sheets which would be free of nickel but which would give much better performance than Type 446.

Now I have invented an alloy steel primarily for rider sheets, but which can be used for other heat treating furnace parts as well, either in wrought or cast form, which is free from nickel; which has excellent resistance to oxidation; and which has much better resistance to stretching under stress at elevated temperatures than Type 446.

Further objects, features and advantages of the invention hereof will appear from the detailed description given below, taken in connection with the accompanying drawings which form a part of the specification and illustrate by way of example, preferred embodiments of the invention.

In the drawings:

Fig. 1 is a longitudinal side elevation view of a normalizing furnace, partially broken away at one end showing the rider sheets and low-carbon steel sheets passing along the rollers thereof;

Fig. 2 is an enlarged transverse sectional elevation of the furnace, as taken at 2—2 of Fig. 1;

Fig. 3 is an enlarged fragmentary perspective showing of a rider sheet supporting a low-carbon steel sheet on the rollers of the furnace; and

Fig. 4 is an enlarged fragmentary perspective showing of a low-carbon steel sheet, sandwiched between a pair of rider sheets.

Referring now in more detail to the drawings and particularly to Figs. 1 and 2 thereof, the normalizing furnace 10, is provided with burners 11 and a hearth 12. The hearth 12 consists of a plurality of longitudinally spaced, parallel shafts 13, rotatably supported above the floor of the furnace in bearings 14, mounted on upstanding supports 15. Each shaft 13 spans the width of the furnace and is provided with a plurality of transversely spaced rollers 16, keyed to the shaft. Suitable motor 55 activated driving means 17, capable of rotating the shafts 13, are located exteriorly of the furnace 10, and thus a series of driven rollers is provided which extends from the inlet end to the exit of the normalizing furnace.

As has been described above, the low carbon steel sheets 18, which are to be normalized, are placed upon rider sheets 19 which in turn are laid upon rollers 16 at the inlet end 20 of the furnace. The driving means 17 imparts rotation to the shafts 13 and rollers 16, whereby the rider sheets together with their associated low carbon steel sheets are then moved toward the exit end 21 of the furnace. As these low carbon steel sheets 18 are thus carried from inlet to exit of the furnace they successively pass through the various heating zones and are thus normalized in the manner that has been pointed out previously. When the sheets reach the exit end 21 of the furnace, they are removed and the low carbon steel sheets are carried to the next processing stage where as

the rider sheets may be loaded upon a cart 22 and returned to the inlet end of the furnace 10 for re-use.

As seen in Fig. 4, in some instances, and especially where the low carbon sheet is made from cold rolled strip, it is desirable not only to support said sheet by rider sheet 19, interposed between the former and the furnace rollers 16, but also to cover said low carbon steel sheet 18 with an additional rider sheet 23 whereby scale formation on the top surface of sheet 18 is minimized.

As has been previously pointed out the work life of these rider sheets is dependent upon the type of steel of which they are made, with steels of ferritic structure being far less advantageous than those of austenitic makings. In order to overcome the aforesaid difficulties which have beset rider sheets of present day steel composition I have developed a substantially austenitic alloy steel which nevertheless is substantially free of any nickel content.

The composition of the steel of my invention is as follows:

|                 | Broad Range | Preferred Range |
|-----------------|-------------|-----------------|
| Percent C.....  | .55/.80     | .60/.70         |
| Percent Mn..... | 9.0/15.0    | 11.0/12.0       |
| Percent Si..... | up to 2.5   | 20/1.0          |
| Percent Cr..... | 21.0/27.0   | 23.0/25.0       |
| Percent N.....  | .30/.50     | .35/.40         |

The balance of this steel is substantially all iron except for usual impurities within commercial tolerances, although the steel may include optional additions of up to about 5% in the aggregate of the elements vanadium, tungsten and molybdenum, with none of these being over 2%.

It is desirable to have a minimum of 21% chromium in the steel of the invention to provide adequate resistance to oxidation in the steel at high temperatures. However, the chromium must be kept below about 27% in order to avoid difficulties in fabrication from ingots to sheets, and also to avoid the presence of ferrite in the steel. Since chromium is a strong ferrite former, the more chromium there is in the steel the more difficult it is to maintain the desired austenitic structure in the steel. As has already been mentioned above, steel is much stronger at temperatures over about 1200° F. when its structure is austenite than when its structure is ferrite.

For the reason given above, the other ingredients in the steel in addition to chromium are present primarily to maintain an austenitic structure in the steel. Nickel, as is well known, is very effective in forming and maintaining an austenitic structure in high chromium steels, but since the steel of this invention is designed to be substantially free of nickel, I depend upon additions of other strong austenite formers, namely, carbon, nitrogen and manganese. Of these, carbon and nitrogen are about equally effective, and much more effective than manganese. However, it is necessary to use an appreciable amount of manganese due to the limited solubilities of carbon and nitrogen in the steel. It is desirable also, from the standpoint of fabrication, to limit the carbon and nitrogen contents to maxima of about 0.80% C and about 0.50% N. When the steel contains chromium at about 21% and carbon and nitrogen at about 0.55% and 0.30%, respectively, the steel can be maintained in an austenitic structure with manganese at about 9%. However, when the chromium is at the upper limit of the range, that is about 27%, it is necessary to increase the carbon, nitrogen and manganese contents of the steel.

A quick indication of the relative amount of ferrite in the steel of the invention is obtained by applying a magnet to the steel and observing its relative magnetic susceptibility. The tabulation of Table I below shows a comparison of a number of compositions based on magnetic susceptibility. To put the steels in the most stably austenitic condition, the samples which were tested were

heated to 2150° F. and air cooled. The samples were rated M for strongly magnetic, SM for slightly magnetic, and VSM for very slightly magnetic.

TABLE I  
Relative magnetic susceptibility and Rockwell "C" hardness of C—Mn—Cr—N steels

[All samples air cooled from 2150° F.]

|    | Bar       | C   | Mn   | Cr   | N   | C+N  | Magnetic Susceptibility | Rockwell C |
|----|-----------|-----|------|------|-----|------|-------------------------|------------|
| 15 | 4990..... | .58 | 11.8 | 24.4 | .15 | .73  | M                       | 26         |
|    | 4993..... | .67 | 11.5 | 25.2 | .09 | .76  | M                       | 26         |
|    | 4382..... | .40 | 14.4 | 24.9 | .43 | .83  | M                       | 28         |
|    | 4378..... | .50 | 11.7 | 25.0 | .36 | .86  | M                       | 31         |
|    | 4383..... | .47 | 14.5 | 25.0 | .43 | .90  | M                       | 29         |
|    | 4991..... | .59 | 12.2 | 27.6 | .31 | .90  | M                       | 31         |
| 20 | 4992..... | .55 | 9.3  | 24.9 | .35 | .90  | SM                      | 32         |
|    | 4988..... | .56 | 11.5 | 24.4 | .38 | .94  | VSM                     | 32         |
|    | 4989..... | .59 | 11.8 | 21.8 | .36 | .95  | VSM                     | 32         |
|    | 4379..... | .57 | 11.4 | 24.3 | .39 | .95  | VSM                     | 32         |
|    | 4994..... | .69 | 9.1  | 24.8 | .29 | .98  | VSM                     | 34         |
|    | 4380..... | .65 | 11.5 | 25.2 | .34 | .99  | VSM                     | 34         |
|    | 4384..... | .57 | 14.3 | 24.6 | .45 | 1.02 | VSM                     | 34         |
|    | 4386..... | .72 | 14.3 | 25.1 | .34 | 1.06 | VSM                     | 36         |
|    | 4385..... | .66 | 13.5 | 24.7 | .44 | 1.10 | VSM                     | 36         |
|    | 4381..... | .79 | 11.7 | 25.0 | .40 | 1.19 | VSM                     | 38         |

NOTE.—These steels also contained about 0.3% Si and up to about 0.4% residual Ni.

It is clear from the above that the steel of the invention is substantially non-magnetic or austenitic, when the sum of carbon and nitrogen is a minimum of about 0.92%. It will also be seen that as the sum of carbon and nitrogen increases, the hardness of the annealed steel also increases.

Some high temperature stretch data on the steel of this invention in comparison with the plain chromium steel, Type 446, are shown in Table II below.

TABLE II  
Stretch data at 1400° to 1800° F.

|    | Bar                     | Type                        | Test Temp., °F. | P. S. I. Stress | Amount of Stretch |
|----|-------------------------|-----------------------------|-----------------|-----------------|-------------------|
| 45 | 4377.....               | Type 446 <sup>1</sup> ..... | 1,400           | 8,000           | 5.0% in 1/2 hr.   |
|    | 4379 <sup>2</sup> ..... | This Invention.....         | 1,400           | 15,000          | 0.9% in 20 hrs.   |
|    | 4377.....               | Type 446 <sup>1</sup> ..... | 1,600           | 4,000           | 5.0% in 1/2 hr.   |
|    | 4379 <sup>2</sup> ..... | This Invention.....         | 1,600           | 8,000           | 1.0% in 20 hrs.   |
|    | 4377.....               | Type 446 <sup>1</sup> ..... | 1,800           | 1,000           | 2.0% in 1 hr.     |
|    | 4379 <sup>2</sup> ..... | This Invention.....         | 1,800           | 1,000           | 0.5% in 20 hrs.   |
|    | 4384 <sup>2</sup> ..... | do.....                     | 1,800           | 1,000           | 0.7% in 20 hrs.   |
|    | 4381 <sup>2</sup> ..... | do.....                     | 1,800           | 1,000           | Do.               |

<sup>1</sup> 0.29 C; 0.5 Mn; 24.4 Cr; 0.23 N.

<sup>2</sup> See Table I for compositions.

Thus it is seen that the steel of this invention is much more resistant than Type 446 to stretching over the temperature range 1400° to 1800° F.

That the oxidation resistance of the steel of this invention is of high magnitude is shown by the data of the following Table III.

TABLE III  
Scale resistance of steels at 2100° F.

|    | Bar       | Type                | Weight Loss After 200 Hrs. At Temperature With Intermittent Cooling to Room Temperature, Grams per sq. in. |
|----|-----------|---------------------|------------------------------------------------------------------------------------------------------------|
| 65 | 5307..... | Type 310.....       | 0.17-0.18                                                                                                  |
|    | 4377..... | Type 446.....       | 0.67-0.74                                                                                                  |
|    | 4379..... | This Invention..... | 0.44-0.48                                                                                                  |
|    | 4384..... | do.....             | 0.45-0.52                                                                                                  |
|    | 4386..... | do.....             | 0.46-0.50                                                                                                  |
|    | 4381..... | do.....             | 0.73-0.82                                                                                                  |

NOTE.—See Table I for composition.

What is claimed is:

1. A rider sheet for use in normalizing furnaces and the like made of a substantially austenitic and substantially nickel free alloy steel having a relatively high resistance to deformation under stress at high temperatures and high resistance to oxidation at temperatures up to about 2100° F., said steel containing about: 21 to 27% chromium; 9 to 15% manganese; 0.55 to 0.8% carbon and 0.3 to 0.5% nitrogen, the sum of carbon and nitrogen being not less than about 0.92%; up to about 2.5% silicon; up to about 5% in aggregate of at least one element selected from the group consisting of vanadium, tungsten, and molybdenum with no one of these being over 2%; and the balance substantially all iron.

2. A rider sheet for use in a furnace for normalizing low carbon steel sheet, said rider sheet being made of substantially austenitic and substantially nickel free alloy steel having a relatively high resistance to deformation under stress at high temperatures and a high resistance to oxidation at temperatures up to about 2100° F., said steel containing about: 23 to 25% chromium; 11 to 12% manganese; 0.6 to 0.7% carbon and 0.35 to 0.4% nitrogen; up to about 2.5% silicon; up to about 5% in aggregate of at least one element selected from the group consisting of vanadium, tungsten, and molybdenum with no one of these being over 2%; and the balance substantially all iron.

3. A rider sheet for use in a furnace for normalizing low carbon steel sheet, said rider sheet being made of a

substantially austenitic and substantially nickel free alloy steel having a good resistance to deformation under stress at high temperatures and a high resistance to oxidation at temperatures up to about 2100° F., said steel containing about: 21 to 27% chromium; 9 to 15% manganese; 0.55 to 0.8% carbon and 0.3 to 0.5% nitrogen, the sum of carbon and nitrogen being not less than about 0.92%; up to about 2.5% silicon; and the balance iron.

4. A rider sheet for use in a furnace for normalizing low carbon steel sheet, said rider sheet being made of a substantially austenitic and substantially nickel free alloy steel having a good resistance to deformation under stress at high temperatures and good resistance to oxidation at temperatures up to about 2100° F., said steel containing about: 23 to 25% chromium; 11 to 12% manganese; 0.6 to 0.7% carbon; 0.35 to 0.4% nitrogen, up to about 2.5% silicon; and the balance iron.

References Cited in the file of this patent

|         |                       |                              |
|---------|-----------------------|------------------------------|
| 20      | UNITED STATES PATENTS |                              |
|         | 2,212,495             | De Vries _____ Aug. 27, 1940 |
|         | 2,380,854             | Lorig _____ July 31, 1945    |
|         | 2,496,247             | Jennings _____ Jan. 31, 1950 |
| 25      | 2,698,785             | Jennings _____ Jan. 4, 1955  |
|         | FOREIGN PATENTS       |                              |
| 152,291 | Austria _____         | Jan. 25, 1938                |